

## UNITED STATES PATENT OFFICE

2,482,517

## CORROSION INHIBITING COMPOSITION

Knapel F. Schliermeier, Alton, and Walter E. Heinz, Roxana, Ill., assignors to Shell Development Company, San Francisco, Calif., a corporation of Delaware

No Drawing. Application March 13, 1945,  
Serial No. 582,582

19 Claims. (Cl. 252—33.4)

**1** This invention relates to new and improved corrosion preventive oils and greases. It particularly pertains to solution-stable mineral oil compositions containing dissolved amounts of certain organic polyhydric alcohols which provide an unusual degree of protection against corrosion to ferrous metals and also against corrosion of other metals and alloys such as copper, brass, bronze, zinc, cadmium, aluminum, magnesium, etc.

It has been found that certain partially esterified polyhydric alcohols wherein the ratio of free hydroxyl to ester radicals is at least 1:1, and preferably greater than 1:1 exhibit anti-corrosive properties when applied to metallic surfaces in solution of hydrocarbon oils. However, this discovery by itself is of little practical value since frequently these compounds have very limited solubilities in hydrocarbons, particularly at relatively low temperatures at which rustproofing oils may have to be used. Thus, the solubility of glyceryl mono oleate in a refined mineral oil at 75° F. is about .25%, at 70° F. about 1%, and at 50° F. immeasurably small. To enable the dissolution of effective amounts, mutual solvents are required.

A considerable number and variety of substances have been evaluated as mutual solvents in attempts to overcome this difficulty but have been found unsatisfactory for one or more reasons. Thus, the addition of amines does not produce satisfactory solution stability and frequently decreases the oxidation stability of the organic medium, oil-soluble alcohols decrease the corrosion protection in addition to yielding unstable solutions, oleic acid and other normally liquid fatty acids increase the solubility of the dihydroxy alcohols in mineral oil but greatly reduce their rust inhibiting potency, etc.

It has been discovered, however, that this problem may be solved in a highly satisfactory manner by the employment of salts, in particular the ammonia, alkali and alkali earth metal salts of oil-soluble organic sulfonic acids. Certain oil-soluble sulfonic acids are known as mahogany acids as distinguished from green acids or water-soluble sulfonic acids and are most readily obtained as a by-product from the treatment of petroleum (for example, lubricating oil fractions) with sulfuric acid. However, oil-soluble sulfonic acids may also be obtained from the treatment of many other organic compositions such as alkyl benzenes, alkyl naphthalenes, coal tars, etc. with concentrated sulfuric acid, or by treatment of aliphatic or cycloaliphatic compounds such as  $C_{10}$  and higher hydrocarbons with chlor sulfonic acid,

**2** Oil-soluble sulfonates of dicarboxylic acid esters such as malonic acid esters represent still another type.

While many of these organic sulfonates have some discernible corrosion inhibiting properties themselves, they are in many ways greatly inferior to the present polyhydric alcohols as rust inhibitors and are employed in the present application for the chief purpose of maintaining a homogeneous solution of the alcohol in petroleum derived vehicles. Indeed, particularly if used in relatively high concentrations such as are normally required for them to exert their anti-corrosive effect, e. g. about 3% or more, they actually decrease the anti-corrosive effect which would be obtained from the alcohols by themselves if the latter were sufficiently soluble. Consequently, only the amount of sulfonates should be employed which is actually necessary to hold the ester alcohols in solution at the lowest temperature to which the composition will be exposed during storage, transportation or use. Often, a solution which will remain homogeneous at normal room temperature (65–70° F.) is sufficient. In other instances, solution stability at a freezing temperature (32° F.) and lower is desirable.

One reason for the harmful effect of excessive amounts of the sulfonate probably lies in the mechanism of the corrosion inhibition by ester alcohols. This mechanism apparently involves plating out of the alcohol from its solution on the metal surface. The closer the solution is to its saturation point with respect to the ester alcohol, the more easily is the latter plated out. For this reason, the ester alcohol must be only little soluble in the hydrocarbon medium, and in general best results are obtained with ester alcohols whose solubility at normal room temperature in hydrocarbon oils is below that of effective inhibiting concentrations, so that at least a small amount of mutual solvent is required to produce storage-stable solutions. On the other hand, solubility must not be too low, as otherwise excessive amounts of the sulfonates are required which would interfere with the flow and other properties of the composition. Ester alcohols of relatively high melting points, i. e. about 200° F. or higher, are in general too insoluble to be usable, and for best performance a melting point below about 200° F. is desirable.

The corrosion inhibiting ester alcohols should contain not less than two free OH radicals separated by not more than three intervening atoms. Preferably at least one hydroxyl radical is on a terminal carbon atom but it may be removed from

such terminal carbon atom by as many as three or four atoms. Additional OH radicals may be located near the first two hydroxyl groups. To this alcoholic portion of the molecule there is attached a predominantly hydrocarbon portion containing a number of carbon atoms sufficient to give the molecule a total minimum carbon content of about 12 and preferably about 15 to 46 carbon atoms. This hydrocarbon portion is attached to the alcoholic portion of the molecule through an ester linkage which may be formed between the hydroxy or an acid radical (if there is one) of the polyhydric alcohol on the one hand, and an acid or alcohol respectively on the other. It is desirable that the hydroxyl radicals and ester linkages of the ester alcohol be as close together as possible, at least two hydroxyl radicals being separated from each other by not more than three directly connected atoms and preferably being attached to vicinal carbon atoms. It is advantageous if the several polar groups are attached to directly connected carbon atoms.

It will be seen that the ester alcohols may be derivatives of glycerine, erythritol, penta erythritol, mannitol, sorbitol, sorbitan, etc. The acid (or alcohol, as the case may be) forming the ester with the polyhydric alcohol should have at least about 10, and preferably between about 10 and 40, carbon atoms, in the form of an aliphatic (including cycloaliphatic) radical.

Suitable radicals comprise, for example, capryl, decyl (decanyl), cetroneyl, undecyl, undecenyl, lauryl (dodecyl), tridecyl, myristyl (tetradecyl), myristolenyl, pentadecyl, palmityl (hexadecyl), hypogaetyl, palmitolenyl, therapinyl, oleyl, elaidyl, erucyl, stearyl, abietyl, etc. Radicals such as are contained in the acids obtained from rosin or tall oil as well as in naphthenic (i. e. cycloaliphatic) acids having the requisite number of carbon atoms are also applicable.

The acid which may form the ester with the polyhydric alcohol is preferably a carboxylic acid, although sulfonic, alkyl sulfuric, phosphoric, alkyl phosphoric, etc. acids are also useful.

Adequate corrosion inhibiting quantities of the present ester alcohol are on the order of from about 0.5% or preferably 1% w. up to about 5% or 10% w. depending on the nature of the particular application. Usually a concentration of about 2%-3% w. is satisfactory. By the designation "% w." is meant the per cent by weight of the additive based on the weight of the medium. The amount of the sulfonate used, depending on its solubility in the particular petroleum medium involved, the solubility of the ester alcohol in the petroleum medium, and the solubility of the ester alcohol in the sulfonate, may vary from about 3 times to  $1/20$  and preferably about  $1\frac{1}{2}$  times to  $1/15$  that of the ester alcohol. Usually the solubility of these alcohols is greater in relatively aromatic as well as more viscous petroleum fractions than in relatively paraffinic and/or lighter oils.

The hydrocarbon medium employed to disperse the ester alcohols is preferably a liquid, although it may be a solid or plastic such as paraffin, petroleum or soap-thickened grease. It is desirable that asphaltenes or resinous constituents of crude petroleum be absent, since they may interfere with the rust protection of the ester alcohols; hence the media comprise generally refined mineral oil or fractions thereof. Refining may be by percolation, sulfuric acid treatment, extraction with selective solvents, propane precipitations, etc. The particular fraction of re-

fined mineral oil which is employed will of course vary with the specific application. If it is desired to produce a rust-inhibiting lubricant for an internal combustion engine the present additives will be incorporated in a lubricating oil which otherwise meets the requirements, such as viscosity, viscosity index, pour point, volatility, color, etc., for this use. On the other hand, if a general utility or instrument oil is required, the additives will be added to an oil of lower viscosity as the case may require, for example having a viscosity at 100° F. of 10-25 cs. The compositions of this invention may be applied to metal surfaces by rolling, dipping, brushing, spraying, swabbing, trowelling, etc.

A number of specific embodiments of the invention follow:

#### Example I

20 A general preservative lubricant meeting the requirements of U. S. Army Ordnance specification AXS-674 (Rev. 2) was made by adding to a refined mineral lubricating oil of 20 API gravity and 740 S. U. S. viscosity at 100° F., 4.5% w. of glycerol mono oleate and 0.5% w. of a 50% concentrate of sodium salt of mahogany acids. This composition afforded protection to a steel strip for 400 hours in the humidity cabinet at 100° F.

#### Example II

30 A coating composition for hot application to metal parts was compounded from 46% w. of 120 penetration aromatic petroleum extract, 46% w. short residue petrolatum, 5% w. neutral, high V. I. lubricating oil, 2.7% w. glycerol mono oleate and 0.3% w. of a 50% concentrate of sodium salt of mahogany acids. It had a melting point of 146° F. and gave protection in the humidity cabinet for over 1000 hours. If desired, this composition may be diluted with mineral spirits or naphtha and applied to the metal at room temperature by dipping, brushing or spraying.

#### Example III

45 To a solvent-extracted light spray oil was added 1.5% w. glycerol mono oleate, 2% w. commercial pour depressor, 0.2% w. tertiary butyl para cresol as anti-oxidant, and 1.5% w. of a 50% concentrate of sodium salt of mahogany acids. 50 This met the requirements for a small arms lubricant of U. S. Army Ordnance specification AXS-777, affording humidity cabinet protection at 100° F. for 200 hours.

#### Example IV

55 A rust-inhibiting instrument oil meeting U. S. Government specification AN-O-6a was prepared by dissolving in an acid treated neutral distillate oil having a viscosity at 100° F. of about 8 centistokes the following additives:

Sorbitan mono stearate ----- 1.75% w.  
Sodium sulfonate (oil-soluble) ----- 2.5% w.  
2,6-ditertiary butyl-6-methyl phenol  
(oxidation inhibitor) ----- .3% w.  
65 Pour point and viscosity improvers ----- 3.0% w.

#### Example V

The harmful effect of excessive amounts of the sulfonate is well demonstrated by the following comparisons: Two solutions of 3% sorbitan mono stearate in a light lubricating oil were prepared, one containing  $1\frac{1}{2}$ % and the other 3% oil-soluble sodium sulfonate. Steel panels coated with these oils had lives of 750 and 500 hours, 75 respectively. Similar solutions using sorbitan

mono palmitate instead of the stearate gave lives of 650 and 450 hours, respectively.

The effect of high solubility of the alcohol ester is shown by the comparison below:

Two solutions in a light lubricating oil with 3% each of sorbitan trioleate and sorbitan monooleate were made. The former was completely soluble. The latter was incompletely soluble. The relative lives in the humidity cabinet of steel panels treated with the solution were 72 and 10 300 hours, respectively.

We claim as our invention:

1. A homogeneous, storage-stable solution in an essentially hydrocarbon medium of a corrosion-inhibiting amount of a partial ester of an acyclic polyhydric alcohol an aliphatic acid having from 10 to 40 carbon atoms, said partial ester having the following properties: a melting point below about 200° F., a solubility in said medium below that enabling dissolution of said amount at normal room temperature in the absence of a mutual solvent, a ratio of hydroxyl to ester radicals of at least 1:1, a content of at least 12 carbon atoms and of at least 2 hydroxyl radicals separated from each other by not more than 3 directly connected atoms, said solution additionally containing an oil-soluble salt of an organic sulfonic acid in an amount sufficient to maintain the ester in solution under normal storage conditions.

2. A homogeneous, storage-stable solution in an essentially hydrocarbon medium of a corrosion-inhibiting amount of a partial ester of an acyclic polyhydric alcohol an aliphatic acid having from 10 to 40 carbon atoms, said partial ester having the following properties: a melting point below about 100° F., a solubility in said medium below that enabling dissolution of said amount at normal room temperature in the absence of a mutual solvent, a ratio of hydroxyl to ester radicals of at least 1:1, a content of at least 12 carbon atoms and of at least 2 hydroxyl radicals separated from each other by not more than 3 directly connected atoms, said solution additionally containing an oil-soluble salt of an organic sulfonic acid in an amount sufficient to maintain the ester in solution at about 32° F.

3. A corrosion inhibiting composition comprising, as a carrier, a major amount of a mineral oil having dispersed therein at least 0.5% by weight of a partial ester of an acyclic polyhydric alcohol and an aliphatic acid having from 10 to 40 carbon atoms, said partial ester having at least two free hydroxy radicals separated from each other by not more than 3 directly connected atoms and having a melting point below about 200° F., said partial ester being solubilized in the mineral oil by addition thereto of an oil-soluble salt of petroleum sulfonic acid, varying in amounts of from about 1½ times to about 1/15 of the partial ester.

4. A corrosion inhibiting composition comprising as a carrier a major amount of a hydrocarbon medium having dispersed therein at least 0.5% and up to about 10% by weight of a glycerol monoester and a minor amount sufficient to solubilize said glycerol monoester of an oil-soluble salt of petroleum sulfonic acid.

5. A corrosion inhibiting composition comprising a major amount of a mineral oil and at least 0.5% and up to about 10% by weight (based on the mineral oil) of a glycerol monoester and an oil-soluble salt of petroleum sulfonic acid added in amounts of from 1½ times to about 1/15 of the glycerol monoester.

6. A corrosion inhibiting composition comprising a major amount of a mineral oil and at least 0.5% and up to about 10% by weight (based on the mineral oil) of a glycerol monooleate and an oil-soluble salt of petroleum sulfonic acid added in amounts of from 1½ times to about 1/15 of the glycerol monooleate.

7. A corrosion inhibiting composition comprising a major amount of a mineral oil and at least 0.5% and up to about 10% by weight (based on the mineral oil) of glycerol mono naphthenate and an oil-soluble salt of petroleum sulfonic acid added in amounts of from 1½ times to about 1/15 of the glycerol mono naphthenate.

8. A corrosion inhibiting composition comprising a major amount of a mineral oil and at least 0.5% and up to about 10% by weight (based on the mineral oil) of a glycerol monoester and an oil-soluble salt of petroleum sulfonic acid added in amounts of from 1½ times to about 1/15 of the glycerol monoester and a minor amount of an alkyl phenolic anti-oxidant.

9. A corrosion inhibiting composition comprising a major amount of a mineral oil and at least 0.5% and up to about 10% by weight (based on the mineral oil) of a glycerol monooleate and an oil-soluble salt of petroleum sulfonic acid added in amounts of from 1½ times to about 1/15 of the glycerol monooleate and a minor amount of an alkyl phenolic anti-oxidant.

10. A homogeneous, storage stable solution in an essentially hydrocarbon medium of a corrosion inhibiting amount of a glycerol mono ester, the acid radical having 10 to 40 carbon atoms, said solution additionally containing an oil-soluble alkali metal salt of an organic sulfonic acid, in an amount sufficient to maintain the ester in solution under normal storage conditions.

11. A homogeneous, storage stable solution in an essentially hydrocarbon medium of a corrosion inhibiting amount of a glycerol mono ester of a fatty acid having from 10 to 40 carbon atoms, said solution additionally containing an oil-soluble alkali metal salt of an organic sulfonic acid, in an amount sufficient to maintain the ester in solution under normal storage conditions.

12. A homogeneous, storage stable solution in an essentially hydrocarbon medium of a corrosion inhibiting amount of a glycerol mono-oleate, said solution additionally containing an oil-soluble alkali metal salt of an organic sulfonic acid, in an amount sufficient to maintain the ester in solution under normal storage conditions.

13. A homogeneous, storage stable solution in an essentially hydrocarbon medium of a corrosion inhibiting amount of a glycerol mono naphthenate, said solution additionally containing an oil-soluble alkali metal salt of an organic sulfonic acid, in an amount sufficient to maintain the ester in solution under normal storage conditions.

14. A homogeneous, storage stable solution in an essentially hydrocarbon medium of a corrosion inhibiting amount of a partial ester of an acyclic alcohol having from 3 to 6 carbon atoms and an aliphatic acid having from 10 to 40 carbon atoms in which each available carbon atom of said alcohol has one hydroxy group attached thereto, said solution additionally containing an oil-soluble alkali metal salt of an organic sulfonic acid, in an amount sufficient to maintain the ester in solution under normal storage conditions.

15. A corrosion inhibiting mineral oil composition comprising a major amount of mineral oil as a carrier, a minor amount, sufficient to inhibit corrosion of a glycerol monoester of a monocarboxylic acid containing at least 10 carbon atoms and a minor amount sufficient to solubilize said glycerol monoester of an oil-soluble sulfonate.

16. A homogeneous, storage stable solution in an essentially hydrocarbon medium of a corrosion inhibiting amount of a glycerol mono-oleate, said solution additionally containing an oil-soluble alkaline earth metal salt of an organic sulfonic acid, in an amount sufficient to maintain the ester in solution under normal storage conditions.

17. A homogeneous, storage stable solution in an essentially hydrocarbon medium of a corrosion inhibiting amount of a partial ester of an acyclic alcohol having from 3 to 6 carbon atoms and an aliphatic acid having from 10 to 40 carbon atoms in which each available carbon atom of said alcohol has one hydroxy group attached thereto, said solution additionally containing an oil-soluble alkaline earth metal salt of an organic sulfonic acid, in an amount sufficient to maintain the ester in solution under normal storage conditions.

18. A homogeneous, storage stable solution in

5 an essentially hydrocarbon medium of a corrosion inhibiting amount of a partial ester of an acyclic alcohol having from 3 to 6 carbon atoms and an aliphatic acid having at least 10 carbon atoms, said solution additionally containing an oil-soluble sulfonate in an amount sufficient to maintain the ester in solution under normal storage conditions.

10 19. A homogeneous, storage stable solution in an essentially hydrocarbon medium of a corrosion inhibiting amount of a partial ester of an acyclic polyhydric alcohol, said solution additionally containing an oil-soluble sulfonate, in an amount sufficient to maintain the ester in solution under normal storage conditions.

KNAPEL F. SCHIERMEIER.  
WALTER E. HEINZ.

#### REFERENCES CITED

20. The following references are of record in the file of this patent:

#### UNITED STATES PATENTS

| Number    | Name     | Date          |
|-----------|----------|---------------|
| 2,339,200 | Sowa     | Jan. 11, 1944 |
| 2,345,199 | Hodson   | Mar. 28, 1944 |
| 2,366,817 | Towne    | Jan. 9, 1945  |
| 2,371,333 | Johnston | Mar. 13, 1945 |
| 2,398,193 | Sharp    | Apr. 9, 1946  |